

## UNITED STATES PATENT OFFICE

2,503,969

HIGH-TEMPERATURE LUBRICATING  
GREASE

Harry W. Rudel, Roselle Park, and Arnold J. Morway, Clark Township, Union County, N. J., assignors to Standard Oil Development Company, a corporation of Delaware

No Drawing. Application March 30, 1948,  
Serial No. 18,081

3 Claims. (Cl. 252—42.1)

1

The present invention relates to high temperature lubricating greases and particularly to greases of such type that are stabilized against oxidation. The invention relates further to means for stabilizing high temperature greases and particularly greases containing high percentages of the soaps of high molecular weight fatty oils or glycerides which normally are subject to rapid oxidation. This application is a continuation-in-part of a previous application, Serial No. 513,474, filed December 8, 1943, by the present inventors (now abandoned).

Numerous types of lubricating greases are known, most of them being based upon mineral lubricating oils thickened to a desired consistency by the use of metal soaps of fatty acids and fatty oils. At ordinary temperatures the grease compositions of this general character are not particularly subject to oxidation but for some purposes it is desirable to add to them substances which inhibit oxidations. The prior art contains numerous suggestions for the addition of antioxidants of various types. Thus the patent to Zimmer and Morway, No. 2,360,631, suggests that slightly alkaline greases containing an alkali metal soap of unsaturated fatty acid may be stabilized by addition of a small amount of saturated fatty acid soap or an amphoteric metal. This reference further suggests the use of a small amount of phenyl alpha naphthylamine as antioxidant and it suggests that other conventional addition agents may be added to greases of the type therein described, such as metal deactivators, extreme pressure agents, etc.

The prior art also contains numerous suggestions of compounds and compositions which are said to be useful as metal deactivators, i. e. to inhibit the catalytic effect of certain metals on hydrocarbon fuels and oils. Thus U. S. Patent No. 2,285,878 to White and Walters described the stabilization of various refined and semi-refined hydrocarbon oils by incorporating therein certain copper deactivators. This patent indicates that certain oxygenated hydrocarbons reacted with certain primary amines are useful. In particular the patent shows that diacetyl acetone (or acetyl) ethylene diamine is an effective gum inhibitor in gasoline and, to a lesser extent, dibenzoyl acetone ethylene diamine is also effective.

The present invention involves an improve-

2

ment over that described in the Zimmer and Morway patent which is applicable particularly to greases containing from 0.1 to about 2% excess alkali (as NaOH) along with substantial quantities of the alkali metal (especially sodium) soaps of fatty oils (glycerides). The excess alkali is added to enhance high temperature stability. Soaps of the fatty oils are to be distinguished from the soaps of fatty acids. The invention also relates to the use of dibenzoyl acetone condensed with a lower alkylene diamine as a potent stabilizer.

As is well understood by those skilled in the art, the saponification of fatty oils results in the release of glycerin from the oil which, where the soap is formed in the oil, remains in the grease, unless particular steps are taken to remove the glycerin. While glycerin per se is not objectionable in greases, it does have a pronounced tendency to promote oxidation and this is particularly true at higher temperatures. Hence, such a grease containing both free or excess alkali and the alkali metal soaps of fatty oils or glycerides tends to have poor resistance to oxidation, especially at higher temperatures. This is particularly true of greases having a high soap content and such greases have been found very difficult to inhibit effectively against oxidation under some conditions.

30 Oxidation in lubricating greases is especially objectionable because it results in the development of acidic bodies predominantly of low molecular weight which are definitely corrosive. This is particularly true of those greases which 35 are designed for lifetime lubrication of ball bearings and the like or for any long continued use. A minor oxidation of a grease which is frequently replaced may be of no consequence, whereas oxidation in a grease that is intended to lubricate a 40 bearing for "life" may be a very serious matter. Certain types of greases based upon the use of substantial proportions of the sodium and/or lithium or other alkali soaps of fats or fatty oils, for example, the unsaturated non-drying vegetable or animal fats and oils having 12 to 22 carbon atoms such as rape seed oil, mustard oil and the like. These have proved very suitable for long time or life time lubrication of bearings where the temperatures may become very high, provided they can be prevented from oxidizing. A 45 specific object of the present invention is to sta-

bilize such compositions over a long period of time. It applies particularly to those greases which are alkaline or contain an excess of saponifying agent. A more particular object is to stabilize them against oxidation at high temperatures. These and other objects will become more apparent as this description proceeds.

According to the present invention, it has now been found that the addition of the combination of an aliphatic acyl acetophenone condensation product such as dibenzoyl acetone with a lower alkylene diamine and an oxidation inhibitor in an amount ranging from 0.1-1% thoroughly stabilizes an alkaline soap base grease of high soap content, e. g. 20 to 40% soap by weight, against rapid deterioration at high working temperatures. Before addition to the grease, these aliphatic acyl acetophenone-alkylene diamine condensation products and the oxidation inhibitor may be compounded to any desired ratio, but it is preferred to utilize about equal parts by weight of anti-oxidant and condensation product. The greases may be compounded in the usual way, such as by melting the high molecular weight fatty acids or corresponding fats in a mineral lubricating oil and while in the molten state either neutralizing the high molecular weight fatty acid or saponifying the corresponding fat with the desired hydrated metallic oxide using an excess of the hydrated oxide over that theoretically required for the reaction. At this point, the grease should be tested for free alkalinity and adjusted to contain from 1% to 2.0%, or 0.35%, which latter amount may be preferred, of free alkali calculated as NaOH. After the neutralization or saponification and alkali adjustment steps have been completed and while the grease is in the molten state, the combination of anti-oxidant and acetophenone-ethylene diamine condensation product is incorporated into the molten grease by stirring, if the grease is to be cast into cakes. Otherwise it is preferable to cool the grease in the kettle to temperatures in the range of 300° F. (while stirring), adding the inhibitors in oil solution to prevent any deterioration of the inhibitors at the high molten state temperatures. Also, if desired, the grease may be compounded by melting suitable soaps containing free alkali in the lubricating oil. After the mass is thoroughly fluid, and preferably just prior to its removal from the cooking vessel, the stabilizing agents are stirred into the fluid grease which is then removed from the vessel. The grease additives of the present invention are well-known compounds and the methods of preparing the same are described in the literature. See also the White et al. patent mentioned above.

Among the oxidation inhibitors useful for the purpose of this invention there may be mentioned various alkylated phenols such as tertiary butyl meta cresol; phenol ethers such as the tertiary butyl ether of o-tertiary butyl, p-cresol; or aromatic amines such as phenyl alpha naphthylamine; etc., as representatives of this class of compounds. The other additives, complementary to the antioxidant, is a condensation product, resulting from the reaction between a polyamine, preferably an alkyl diamine and an aliphatic acyl acetophenone. A specific example of this type of compound is di(benzoyl acetyl)-ethylene diamine which may be represented by the formula



Generically this type of condensation product falls within that class of compounds represented by the following empirical formula



in which R represents an aromatic hydrocarbon radical such as phenyl, toluyl, etc., or any homologue thereof; R' represents a monovalent alkyl hydrocarbon radical such as methyl, ethyl, etc., and homologues thereof and R'' represents a bivalent alkylene hydrocarbon radical such as ethylenyl, propylenyl, etc., and homologues thereof. Compounds of this class can be obtained by reacting aromatic acyl-substituted ketones such as benzoyl acetone; methyl benzoyl acetone; ethyl benzoyl acetone; benzoyl methyl ethyl ketone; benzoyl methyl propyl ketone; methyl benzoyl methyl ethyl ketone; ethyl benzoyl methyl ethyl ketone, etc., with alkylene polyamines such as ethylene diamine; 1:2-propylene diamine; 1:3-propylene diamine, diethylene triamine, triethylene tetramine, etc.

In order to show the efficacy of the combination of this invention, the Norma-Hoffman bomb oxidation test for lubricating greases was chosen as the testing medium. The conditions of the test were: 110 pounds per square inch initial oxygen pressure, 210° F. bath temperature, and using copper catalyst (0.25 x 1.75 x 0.015 electrolytic copper sheet). The test was run noting the number of hours required to obtain a 5-pound drop in oxygen pressure. The time required to secure a 5-pound pressure drop is customarily designated as the oxidation induction period and most recent specification includes 100 hours as the minimum oxidation induction period. A grease of the following composition was selected as the testing specimen:

|        |                               |
|--------|-------------------------------|
| 26.00% | rape seed oil                 |
| 0.50%  | sodium sulfonate              |
| 5.63%  | NaOH                          |
| 67.32% | Coastal oil (55 vis./210° F.) |
| 50.50% | phenyl alpha-naphthylamine    |

The results of the Norma-Hoffman test using various additives complementary to the phenyl alpha-naphthylamine antioxidants are shown in the table below:

Table I

|                                                  | No. of Hours<br>for 5# Pressure<br>Drop |
|--------------------------------------------------|-----------------------------------------|
| Grease (blank)                                   | 56                                      |
| Grease + .5% Di-salicyl-ethylene diamine         | 60                                      |
| Grease + .5% Salicyl hydroxamic acid             | 90                                      |
| Grease + .5% Di-acetyl acetyl-ethylene diamine   | 90                                      |
| Grease + .5% Di-benzoyl acetyl-ethylene diamine  | 246                                     |
| Grease + .5% Di-benzoyl acetyl-propylene diamine | 146                                     |

It will be noted that in this particular grease, the only highly effective metal deactivators tested were the dibenzoyl compounds. The disalicyl-ethylene diamine gave substantially no improvement over the blank grease. The salicyclal hydroxamic acid compound and the diacetonyl-ethylene diamine compound gave minor improvement. The latter is indicated in the White et al. Patent No. 2,285,878, as being a very effective gum inhibitor for gasoline, superior to the dibenzoyl compounds. The reverse appears to be true in the type of grease described above.

In view of the foregoing data, which indicated that the dibenzoyl acetone condensed with lower alkylene diamines (ethylene or propylene) was specifically effective in high soap content alkaline grease, the condensation product of dibenzoyl acetone with ethylene diamine being particularly effective, an extensive series of tests was conducted with the results set forth in Table II. The grease in each case was a slightly alkaline grease (about 0.35% as free NaOH) containing approximately 30% by weight of sodium soap of rape seed oil in a Coastal oil of about 55 S. S. U. viscosity at 210° F. The antioxidant used was phenyl alpha naphthylamine. The latter is preferably used in concentrations of 0.1 to 2%, 0.5 to 1% being especially preferred, but in some cases it may be omitted altogether.

5 of at least 0.1% and not more than about 1.0% of the deactivator these percentages being by weight based on the total composition.

The metal deactivators shown in the last three lines of the table were almost if not entirely ineffective, greases containing them showing no improvement over those containing no deactivator whatsoever.

10 The reasons for the specific effectiveness of benzoyl acetone condensed with a lower alkylene diamine are not known. It appears to be clearly established, however, that alkaline greases containing 20% and more, up to 35% or 40% of soaps of fatty oils, saponified in the oil so as to leave glycerine in the composition, present a 15 peculiar problem in deactivation. This is doubtless due in part to their glycerine content (or

Table II

| Antioxi-dant (Wt. Percent) | Oxidation of Alkaline Grease            |  | Hours For Pressure Drop |     |       |       |       |       |       |
|----------------------------|-----------------------------------------|--|-------------------------|-----|-------|-------|-------|-------|-------|
|                            | Metal Deactivator (Wt. Per Cent)        |  | 1#                      | 5#  | 10#   | 15#   | 20#   | 25#   | 30#   |
| 0.5                        | None                                    |  | 56                      | 74  | 86    | 106   | 118   | 130   | ----- |
| 0.5                        | do                                      |  | 37                      | 83  | 107   | 111   | 119   | 133   | ----- |
| 0.5                        | do                                      |  | 8                       | 56  | 92    | 114   | 134   | ----- | ----- |
| 0.5                        | 0.5% Salicylaldehyde+Ethylene Diamine   |  | 18                      | 60  | 86    | 116   | 138   | 160   | 178   |
| 0.5                        | do                                      |  | 16                      | 88  | ----- | ----- | ----- | ----- | ----- |
| 1.0                        | do                                      |  | 36                      | 88  | 132   | 170   | 214   | 230   | ----- |
| 1.0                        | do                                      |  | 18                      | 84  | 131   | 163   | 191   | 215   | ----- |
| 0.5                        | 0.5% Salicylaldehyde+Propylene Diamine  |  | 8                       | 74  | 108   | 134   | 162   | 186   | 202   |
| 0.5                        | 0.5% Salicylhydroxamic Acid             |  | 50                      | 90  | 112   | 134   | 138   | 158   | 160   |
| 0.5                        | 0.5% Isooctyl Salicylhydroxamic Acid    |  | 34                      | 84  | 128   | 158   | 178   | 190   | ----- |
| 0.5                        | 0.5% Acetylacetone+Ethylene Diamine     |  | 26                      | 90  | 106   | 120   | 134   | ----- | ----- |
| 1.0                        | do                                      |  | 84                      | 118 | 134   | 148   | 160   | 178   | ----- |
| 0.5                        | 0.5% Benzoylacetone+Ethylene Diamine    |  | 60                      | 246 | 280   | 294   | 310   | 326   | 334   |
| 0.5                        | do                                      |  | 50                      | 248 | 304   | 320   | 330   | 342   | ----- |
| 0.5                        | 0.2% Benzoylacetone+Ethylene Diamine    |  | 84                      | 148 | 172   | 194   | 210   | 220   | 228   |
| 0.5                        | 0.1% Benzoylacetone+Ethylene Diamine    |  | 110                     | 152 | 176   | 184   | 200   | 214   | ----- |
| 1.0                        | 0.5% Benzoylacetone+Ethylene Diamine    |  | 64                      | 222 | 260   | 274   | 286   | ----- | ----- |
| 1.0                        | 0.1+ Benzoylacetone+Ethylene Diamine    |  | 84                      | 140 | 164   | 178   | 194   | 206   | ----- |
| 0.5                        | 0.5% Benzoylacetone+Propylene Diamine   |  | 80                      | 164 | 190   | 212   | 226   | 234   | 246   |
| 0.5                        | do                                      |  | 84                      | 146 | 170   | 188   | 198   | 214   | 220   |
| 0.5                        | 0.5% Benzoylacetone+Diethylene Triamine |  | 26                      | 64  | 86    | 110   | 128   | 138   | 154   |
| 0.5                        | 0.5% Benzoylacetone+Isobutyl Amine      |  | 14                      | 54  | 82    | 98    | 112   | 122   | 134   |
| 0.5                        | 0.5% Dibenzoylmethane+Ethylene Diamine  |  | 6                       | 60  | 96    | 116   | 136   | 146   | 160   |

It will be noted from the foregoing table that various metal deactivators known in the prior art and used hitherto as successful antioxidants in gasoline, for example, and even in lubricating oils, behaved very differently when used in high soap content grease. It appears from various data that have been obtained that greases containing 20% or more of alkali metal soap of fatty oils (where glycerin is present) are particularly difficult to deactivate or inhibit for high temperature use. The condensation product of salicylaldehyde and ethylene diamine or propylene diamine gave poorer results in some instances than no deactivator. Salicyl hydroxamic acid and isooctyl salicylhydroxamic acid, both of which have been suggested as effective deactivators, gave little or no improvement. Acetyl acetone condensed with ethylene diamine, indicated in the prior art to be an effective inhibitor for gum in gasoline, showed no appreciable improvement. Even where the quantity of antioxidant was increased to 1.0%, the improvement was only moderate.

On the other hand, the condensation product of benzoyl acetone and ethylene diamine was very effective in a concentration of 0.5% and even in concentrations as low as 0.1% it showed a greater oxidation life for a 5 lb. drop in oxygen pressure than 0.5% of any of the other metal deactivators. The related propylene diamine derivative also showed up pretty well, both being substantially superior in the 5 lb. drop test which is the most significant, to all other metal deactivators. This invention contemplates the use

derivatives thereof) and may be due in part also to the free alkali which is present.

45 It will be understood, therefore, that the invention contemplates the use of a specific type of stabilizer for alkaline greases of high soap content where the soap is formed from fats or glycerides. It has specific application to those 50 greases containing about 20% or more by weight of the alkali metal soaps of rape seed oil and related unsaturated oils. The lubricating oil may vary in viscosity and in viscosity index and various other additives such as stringiness and tackiness agents, extreme pressure agents, etc., 55 may be included as will be apparent to those skilled in the art.

What is claimed is:

1. A lubricating grease composition consisting essentially of mineral base lubricating oil containing 20 to 40% by weight of the sodium soap of rapeseed oil, said composition having a substantial glycerine content and a content of 0.25 to 2% excess alkali calculated as free sodium hydroxide, 0.1 to 2% phenyl alpha naphthylamine, and 0.1 to 1% of dibenzoyl acetone alkylene diamine wherein the alkylene group is selected from the group consisting of ethylene and propylene.
2. A lubricating grease composition consisting essentially of mineral base lubricating oil, about 30% by weight of sodium soap of rape seed oil said composition having a substantial glycerine content and having excess alkalinity of about 0.35% calculated as free sodium hydroxide, 0.5

to 1% phenyl alpha naphthylamine, and 0.1 to 0.5% dibenzoyl acetone ethylene diamine.

3. A lubricating grease composition consisting essentially of mineral base lubricating oil, about 30% by weight of sodium soap of rape seed oil said composition having a substantial glycerine content and having excess alkalinity of about 0.35%, calculated as free sodium hydroxide, 0.5 to 1% phenyl alpha naphthylamine, and 0.1 to 0.5% dibenzoyl acetone propylene diamine.

HARRY W. RUDEL.  
ARNOLD J. MORWAY.

## REFERENCES CITED

The following references are of record in the file of this patent:

## UNITED STATES PATENTS

| Number       | Name             | Date          |
|--------------|------------------|---------------|
| 2,265,791    | Zimmer et al.    | Dec. 9, 1941  |
| 2,285,878    | White et al.     | June 9, 1942  |
| 2,289,748    | Beerbower et al. | July 14, 1942 |
| 10 2,340,438 | Strawn           | Feb. 1, 1944  |
| 2,360,631    | Zimmer et al.    | Oct. 17, 1944 |